

## UNITED STATES PATENT OFFICE

1,973,907

MANUFACTURE OF REFRACtORY BRICKS  
OR THE LIKE FROM CHROME ORE

Elisabeth Lux, Essen-Ruhr, Germany, assignor,  
by mesne assignments, to The Koppers Company  
of Delaware, Pittsburgh, Pa., a corporation of  
Delaware

No Drawing. Application January 25, 1932,  
Serial No. 588,829. In Germany January 24,  
1931

6 Claims. (Cl. 25—156)

(Granted under the provisions of sec. 14, act of  
March 2, 1927; 357 O. G. 5)

I have filed an application in Germany on  
January 24, 1931.

The invention relates to the manufacture of  
refractory bricks and more particularly to the  
manufacture of refractory bricks or the like from  
chrome ore.

It is well-known that the commercial chrome  
bricks generally suffer from their inability to sup-  
port loads at high temperatures. It also is known  
10 that the ordinary chrome bricks only possess a  
low spalling resistance. One has already tried to  
improve the quality of chrome ore bricks by add-  
ing to the refractory mass used for the manu-  
facture of chrome ore bricks certain substances.  
15 For instance from mixtures of chrome ore and  
diaspore, bricks with relatively favourable qual-  
ities have been manufactured, which are better  
able to withstand any sudden change of temper-  
ature than bricks made from chrome ore.

20 The first object of my present invention is to  
provide an improved method for making chrome  
ore bricks by which it is rendered possible to man-  
ufacture chrome ore bricks which are not only  
able to stand better rigid thermal change but also  
25 show an improved load bearing capacity at high  
temperatures.

A further object of my present invention is to  
provide an improved refractory mass suitable for  
the manufacture of highly refractory chrome  
30 bricks, which are able to stand better sudden  
changes of temperatures and show an improved  
load bearing capacity at high temperatures.

Finally, an object of my invention is refrac-  
tory bricks or the like from chrome ore, which  
35 are able to stand better sudden changes of tem-  
perature and show an improved load bearing ca-  
pacity at high temperatures.

With these and other objects of my invention  
in view I will now describe the nature of my  
40 present invention more fully in details.

I have found that certain slags which are re-  
covered as waste products from the manufacture  
of ferro-chromium and ferro-vanadium by the  
so-called thermite-process in a proportion of 10  
45 to 40 per cent added to the chrome ore mass are  
suitable to raise essentially the softening point of  
chrome ore bricks under a load of about 50 lbs.  
per sq. inch, whereby at the same time the abil-  
ity of the bricks to withstand changes of tem-  
50 peratures is considerably increased.

Refractory bricks made of chrome ore alone  
generally fail suddenly under load of 50 lbs. at  
1450° C. or less. This temperature could be raised  
by an addition of 10% of the above mentioned  
55 slags to about 1570° C., by an addition of about

20% to about 1650° C. and by an addition of  
30% of the above mentioned slags above 1700° C.  
The herein mentioned indications of temperature  
refer to degrees centigrade.

The slag used by me as an addition to the  
chrome ore has generally a content of approxi-  
mately 73%  $Al_2O_3$  and about 23%  $MgO$  together  
with a small quantity of other constituents. The  
percentage of  $SiO_2$  in slag amounts to 1% or less.

I have further found that one can obtain the  
same effect when making a chrome ore brick as  
with a slag from the ferro-chrome and ferro-  
vanadium production also with other kinds of  
slag which contain only a small percentage of  
silica and up to 90% or more of  $Al_2O_3 + MgO$   
60 together or under certain circumstances of  
 $Al_2O_3 + MgO + Cr_2O_3$  together. I wish to char-  
acterize those kinds of slag which are suitable of  
employment in the case of my present invention  
65 for the improvements of the quality of chrome  
ore bricks in that the slag must consist essen-  
tially of magnesia-alumina compounds, possibly  
also of chromium compounds, of which the con-  
70 tents of magnesia may be lower than in the case  
of the corresponding spinel compound.

As to the percentage of slag in the manufac-  
ture of chrome ore bricks in single cases, this  
depends on to what degree of resistance against  
heat the ready bricks should have or up to which  
75 point of temperature the chrome ore brick may  
soften under load, any mixture of chrome ore  
and the refractory slag being possible.

80 For instance, according to my present inven-  
tion, one may proceed to the manufacture of  
high refractory and temperature changes re-  
sisting chrome ore bricks as follows:

85 350 kilos chrome ore with about 40%  $Cr_2O_3$   
and 150 kilos of a metallurgical slag with 73%  
 $Al_2O_3$ , 23%  $MgO$  and less than 1%  $SiO_2$  may be  
ground to a grain size under 3 mm. and mixed in  
90 a wet pan with the addition of 4% of water and  
a small quantity of a customary organic cleav-  
ing mixture for instance dextrine. The ready  
mixed mass may be shaped by pressing or in  
95 any other suitable manner and the shapes are  
thereupon dried and finally burned in usual  
manner at temperatures of about 1450° C. to  
100 1500° C. The ready brick can resist under a load  
of 50 lbs. per sq. inch up to a temperature of  
105 about 1700° C.

I wish to be understood that I do not confine  
my invention to the exact details described, but  
that it may be varied within the scope of the  
claims hereinafter made.

60

65

70

75

80

85

90

95

100

105

110

I claim:

1. The method for manufacturing refractory bricks or the like from chrome ore comprising adding to between 90% and 60% of reduced chrome ore of about 40% Cr<sub>2</sub>O<sub>3</sub>, between 10 and 40% of reduced metallurgical slag recovered as a waste product of a metallurgical process and consisting of not less than substantially 90% of magnesia and alumina and not more than 1% of silica, adding further a liquid, moulding the mass into shapes and finally burning said shapes.
2. The method for manufacturing refractory bricks or the like from chrome ore comprising adding to chrome ore metallurgical slag recovered as a waste product of a metallurgical process and consisting of not less than substantially 90% of magnesia and alumina and not more than 1% of silica, adding further a liquid, moulding the mass into shapes, drying said shapes and finally burning same.
3. The method as set forth in claim 2, wherein as addition to the chrome ore the slag used is one which is obtained by the so-called thermite-process for manufacturing ferro-vanadium or ferro-chromium.

4. Refractory mass for the manufacture of highly refractory chrome bricks comprising between 90% and 60% chrome ore of about 40% Cr<sub>2</sub>O<sub>3</sub>, and between 10 and 40% of a metallurgical slag recovered as a waste product of a metallurgical process, said slag consisting substantially of at least 90% of magnesia and alumina and not more than 1% of silica, and a liquid.

5. Refractory mass for the manufacture of highly refractory chrome bricks comprising between 90% and 60% chrome ore of about 40% Cr<sub>2</sub>O<sub>3</sub>, and between 10 and 40% of a metallurgical slag which is obtained as a waste product from the so-called thermite process for the production of ferro-chromium or ferro-vanadium and having a content of about 73% Al<sub>2</sub>O<sub>3</sub> and 23% MgO and not more than 1% of silica, and a liquid.

6. Highly refractory brick made from a mass as described in the claim 5, said mass having been moulded into shapes and finally burned.

ELISABETH LUX.

100

30 105

35 110

40 115

45 120

50 125

55 130

60 135

65 140

70 145

75 150